

## UNITED STATES PATENT OFFICE

2,109,779

## PRESSURE BEARING LUBRICATING OIL

Arnold J. Morway, New York, N. Y., assignor to  
Standard Oil Development Company, a corpora-  
tion of Delaware

No Drawing. Application June 19, 1934,  
Serial No. 731,268

## 10 Claims.

(Cl. 87—9)

The present invention relates to an improved lubricating composition especially for lubrication under high pressure which is encountered in automobile transmissions or other similar mechanisms. The invention will be fully understood from the following description.

In recent years more attention has been continually paid to lubrication of gears, transmission and other mechanisms operating under heavy loads. The use of hypoid gears has increased the need for compounds carrying increased loads at higher speeds. The ordinary compounds used for such service are the so-called "leaded" oils which contain lead oleate.

15 The present invention deals with a new composition for the same general type of service. The composition comprises an oil-soluble zinc salt or soap used in connection with a material rich in sulphur, both of these ingredients being 20 incorporated in a high grade hydrocarbon lubricating oil. As a particularly desirable modification of the broader idea is contemplated a mixture of both lead and zinc soaps along with the sulphur compound which is much superior 25 to other compounds with respect to the load bearing capacity at high speeds, and particularly with regard to the appearance and condition of the gear teeth and other metal parts.

30 The zinc salts which are used in the present composition comprise the usual soaps or salts of the high molecular weight organic acids such as oleic, stearic, and mixtures of the same such as may be obtained from tallow and other natural fats. In addition to these commercial fatty 35 acids may be mentioned certain organic acids which are particularly interesting to the petroleum refiners in that they are directly obtainable from petroleum. Among these are included the oil soluble sulphonic acids, those obtained by 40 treating lubricating oils, cracked wax, or other such material with sulphuric acid, especially with concentrated or fuming acid, as in the manufacture of petroleum white oils. Certain alkyl sulphuric acids may also be used, particularly those 45 in which the alkyl group contains at least 10 carbon atoms, and may be obtained by the sulphation of cracked or unsaturated paraffin wax. It is to be understood that these alkyl sulphuric acids are mono-alkyl products of which the 50 alkyl group may be either primary, secondary or tertiary. The other hydrogen atom of the acid is to be combined with the zinc salt in the usual manner. Napthenic acids are also contemplated such as are obtained from Roumanian, Russian 55 and certain domestic crude oils either in the

natural or cracked condition. Furthermore, certain synthetic acids are also contemplated such as are obtained by the oxidation of paraffin wax at relatively low temperatures with air or other oxidizing agents.

5 The soaps may be made in any desirable manner, for example, by adding metallic oxide directly to the fatty or other soap acid, and raising the temperature to bring about reaction, or in an alternative manner by adding inorganic 10 salts of the particular metals, for example, zinc chloride to soda soaps so as to form the heavy metal soap by double decomposition. The soaps are added in the present compositions to the extent of 10 or 20% so as to furnish from 2 to 5% 15 of the metal in final composition. If lead soaps are to be used in combination with the zinc soaps as preferred then they may be used in equimolar proportions, or more or less of either the one or the other may be used, for example, 3 20 mols of lead to 1 mol. of zinc or vice versa. The mixture of the two metals ordinarily gives much better results than either alone.

25 The sulphur compounds that are used in the present compositions are of a type of oil-soluble organic sulphur compounds, and may be obtained from certain sulphur rich crudes especially found in East Texas fields. Corrosive sulphur is preferred to the non-corrosive types and the word "corrosive" is used in a special sense to 30 describe that type of compound, including free sulphur, which is capable of discoloring a bright copper strip when applied according to the method ordinarily used for testing gasoline and described by the American Society for Testing Materials.

35 The corrosive compounds should be sufficiently high boiling so as not to be lost by evaporation, and pure compounds may be used instead of the naturally occurring sulphur which was referred 40 to above, for example, high molecular weight mercaptans, polysulphides, preferably trisulphide or higher, as well as free sulphur itself, which may be added in small amounts. Olefines, for example, obtained from cracked wax, or vegetable, mineral and marine oils may also be sulphurized by cooking with free sulphur or sulphur chloride and sulphurized terpenes, such as sulphurized pine oil may also be employed. The amount of the corrosive sulphur in the final 45 composition is preferably from about .3 to about 1%, and the best results are obtained by having this amount of truly corrosive sulphur in addition to any amount of non-corrosive sulphur which might be present. The amount of truly corrosive 50 sulphur is not to be exceeded by more than 55

sulphur can be determined as the difference between total sulphur determinations before and after heating with a finely divided metal such as copper.

5 The oils to which the heavy metal soaps are added should be well refined mineral lubricating oils either heavy distillates or residuals, cylinder stocks and the like. They may be obtained from various crudes refined by acid and clay in the 10 usual manner or by solvent extraction, hydrogenation, destructive hydrogenation and similar processes. It has been found that all of the metallic soaps are not readily soluble in all types of mineral oils, especially in the high quality base 15 oils, that is to say, those which have viscosity indices of 70 or 80 and above. In the low quality oils having a viscosity index below about 50 any of the various soaps may be used without difficulty. In the higher quality oils, however, 20 special treatment may sometimes be necessary. For example, the oil may be given a light oxidation treatment with air which for unknown reasons renders it capable of dissolving the various soaps. On the other hand, special soluble 25 soaps can be used and among these the lead and zinc naphthenates and sulphonates are probably the most desirable.

In describing these metallic compounds it has been indicated that lead and zinc soaps may be 30 added to the composition. These soaps may be pre-formed in each case and separately added or a mixed soap may be prepared which may be either a mixture of the two soaps or may be a double soap in which the lead and zinc materials are both present in chemical combination. 35 Other addition agents may be present without detriment, for example thickening agents, oxidation and pour point inhibitors, dyes for color or cast, chlorine compounds, esters, alcohol and 40 the like for increased oiliness.

#### Example I

In the following tests the same base oil is used and the tests were all conducted in the same 45 manner on the Almen machine. This machine and test method have been described in Nat. Pet. News of Nov. 11, 1932. The data is as follows:

| 50 | Oil sample                                                           | Load carried<br>#/sq. in. | Final<br>friction<br>in<br>pounds | Load at<br>which<br>fric. rises<br>suddenly | Max.<br>temp. | Pin<br>condition          | 50 |
|----|----------------------------------------------------------------------|---------------------------|-----------------------------------|---------------------------------------------|---------------|---------------------------|----|
| 55 | 1. Straight hydrocarbon oil.                                         | 3,000                     |                                   |                                             |               | Sheared                   |    |
|    | 2. Same+10% lead naphthenate.                                        | 3,000                     |                                   |                                             |               | Do.                       |    |
|    | 3. Same+10% zinc naphthenate.                                        | 3,000                     |                                   |                                             |               | Do.                       |    |
|    | 4. Same oil sulphurized—1% corrosive sulphur.                        | 15,000                    | 9.0                               | 5,000                                       | 250°          | Scored                    |    |
| 60 | 5. Sulphurized oil (1% S.) 10% zinc naphthenate.                     | 15,000                    | 3.2                               | Smooth<br>curve                             | 130           | Pin<br>bright<br>unscored | 55 |
|    | 6. Sulphurized oil (1% S.) 5% zinc naphthenate, 5% lead naphthenate. | 15,000                    | 3.4                               | Smooth<br>curve                             | 135           | Pin<br>bright<br>unscored | 60 |
| 65 |                                                                      |                           |                                   |                                             |               |                           | 65 |

It is clear from the table that Samples 1, 2 and 3 failed badly and apparently did not increase the load carrying capacity of the oil at all. The final friction was very high, so high in fact as to shear the pin. The fourth sample was much better; it carried the entire test load but the friction curve was not smooth and suddenly mounted at a load of 5000#/sq. in. The 75 final friction was high, much heat was developed

and the pin was scored. Nevertheless it was markedly superior to the prior samples. Samples 5 and 6 showed a still greater improvement. These compositions may have been able to carry even greater loads but 15,000 was the limit of 5 the test. Friction was much lower, the curve was smooth and without any sudden rises and the pin condition was excellently burnished in each case with metallic zinc deposited on the rubbing surfaces of pin and bushing. The heat development was not excessive in either case. 10

#### Example II

To a well refined lubricating oil was added 10% of a sulphurized pine oil and 5% each of lead 15 and zinc naphthenates. The final composition showed the following analysis and specification:

|                    |      |              |
|--------------------|------|--------------|
| Viscosity @ 100° F | 1215 | Sec. Saybolt |
| Viscosity @ 210° F | 95   | Sec. Saybolt |
| Viscosity index    | 90   |              |
| Zinc               | .5%  |              |
| Lead               | 1.5% |              |
| Total sulphur      | .8%  |              |
| Corrosive sulphur  | .3%  | 25           |

In the Almen test this compound carried the full 15,000#/sq. in. The frictional curve with load was smooth throughout with a final frictional value of 3.6 inch pounds. The bearing 30 after test was in excellent condition without any indication of scoring or excessive wear and it had a bright zinc coating.

The present invention is not to be limited by any theory of the mechanism by which the soaps 35 affect the load bearing capacity of the oil nor to any particular acid constituents of such soaps, nor in fact to any particular proportions of soap or soaps in the mixture, nor to any particular oil or sulphur compounds, but only to the following 40 claims in which it is desired to claim all novelty inherent in the invention.

I claim:

1. An improved lubricating composition comprising a viscous petroleum fraction and zinc soap 45 soluble therein, and a corrosive sulphur compound dissolved in said oil.

2. An improved lubricating oil comprising a viscous petroleum hydrocarbon, zinc soap soluble therein, and a corrosive sulphur compound dissolved in said oil.

3. An improved lubricating oil comprising a viscous petroleum fraction and zinc soap soluble therein, and prepared from an acid containing more than 10 carbon atoms selected from the group of fatty acids, unsaturated acids and or 70 75

- ganic acids derived from petroleum, and a corrosive compound of sulphur dissolved in said oil.
4. Composition according to claim 3 in which the zinc soap is derived from an acid obtained from petroleum and selected from the class consisting of naphthenic acids, sulphonic acids, alkyl sulphuric acids and acids derived from the oxidation of paraffin wax.
5. Composition according to claim 3 in which a soluble lead soap is present in addition to the zinc soap.
6. Composition of matter according to claim 3 in which the sulphur is present as a compound selected from the group consisting of high boiling mercaptans, polysulphides and olefines, vegetable, animal and marine oils which have been sulphurized.

7. An improved lubricating composition comprising a viscous petroleum lubricating oil having a viscosity index above 70, zinc naphthenate dissolved therein, and a corrosive sulphur compound dissolved in said oil.

8. Composition according to claim 7 in which lead naphthenate is present in addition to the zinc naphthenate.

9. An improved lubricant comprising a viscous petroleum oil containing soluble zinc soap of an acid selected from the class consisting of naphthenic and sulphonic acids in proportion to give from about 2 to 5% of zinc in the finished lubricant, and a soluble corrosive sulphur compound.

10. Lubricant according to claim 9 in which the mineral oil has a viscosity index above 70.

ARNOLD J. MORWAY.